

## UNITED STATES PATENT OFFICE

2,047,975

PAPER AND PROCESS FOR THE  
MANUFACTURE OF SAMELeo Liberthson, New York, N. Y., assignor to L.  
Sonneborn Sons, Inc., a corporation of Dela-  
wareNo Drawing. Application October 29, 1932,  
Serial No. 640,344

2 Claims. (Cl. 91—68)

The invention is applicable to the impregnation of paper with a copper compound for the purpose of inhibiting or preventing the growth of fungi, etc; and for the purpose of inhibiting or preventing the propagation, passage or transfer of fungi, etc; through the impregnated paper.

The impregnation with a copper compound in aqueous solution has already been practiced, and copper so introduced is known to be efficacious in restricting the growth of fungi. In general, I have found that better results than those obtainable by use of aqueous solutions are obtainable by the process hereinafter described, both as to the amount of copper with which the material 5 may be impregnated and with respect to the efficacy and permanence of retention. In accordance with this process, the copper in the form of an oil soluble copper compound is dissolved in a hydrocarbon and the material is then impregnated with the solution of the copper compound in said hydrocarbon. The hydrocarbons generally 10 may be employed for this purpose, and for certain purposes a hydrocarbon which is normally liquid, such as a lubricating oil derived from petroleum, is preferred. For many purposes, however, a wax-like hydrocarbon is more satisfactory. By the term "wax-like" I wish to comprehend the normally solid or semi-solid hydrocarbons of a waxy character, such as paraffin or petro- 15 latum. For certain purposes, asphalts, wax tailings, etc., may be employed; and such materials, including wax, petrolatum, etc., will be generally referred to as the normally solid hydrocarbons. I may, within the general purview of the invention, employ any oil soluble copper compound, such as copper naphthenate or copper sulphonate, including both the aromatic and aliphatic sulphonates of copper. The preferred 20 material for my process is, generally speaking, a copper soap, viz, a compound of copper with a fatty acid.

A paper impregnated in accordance with my process may be utilized, for example, as a wrapping material in any case where the fungicidal properties of copper are of value. An example of such use is for the purpose of wrapping fruit for storage and/or transportation, in order to minimize the spread of rot (as for example "Botrytis rot") or similar diseases from infected to healthy fruit; the paper so prepared is of course susceptible to other uses. Some paper utilized for this purpose has been heretofore impregnated with copper sulphate. Such paper may, however, become dry and brittle, cracks may occur in the material, or the copper content may be lost as

a result of excessive moisture from any source. The amount of copper which may furthermore be introduced through the heretofore known methods is relatively limited, and is not sufficient under all circumstances to exert the desired fungicidal effect. I have found that superior results are obtainable by the application of the process as hereinbefore described.

It is, of course, desirable that paper for this purpose should contain a substantial percentage 10 of the copper compound, and this in turn requires that the impregnating material shall be correspondingly high in its content of copper carried in solution. The material used for impregnation must, notwithstanding, possess a desirable 15 consistency to permit of easy application and thorough penetration at the temperature of impregnation. I have found that both desiderata may be obtained through the use of a mixture of copper oleate and copper resinate dissolved as 20 aforesaid. This mixture has sufficient solubility in hydrocarbon materials so that a relatively large percentage of combined copper may be introduced to the paper. I preferably employ for this purpose a mixture of copper oleate and copper resinate in which the copper oleate is roughly 25 from 25 to 75% of the total copper soap, and the copper soaps are present in the hydrocarbon to the extent of from 25 to 75% of the whole.

A still further improvement results from the 30 preliminary formation of the copper soap by the metathetical reaction in the presence of water between a water soluble soap and a water soluble copper compound. The copper soap may, for example, be made by reacting a sodium soap with 35 copper sulphate. If this reaction is carried out in the presence of the hydrocarbon, the copper soap will be found at the expiration of the reaction dissolved in the hydrocarbon. Where a wax-like or normally solid hydrocarbon is employed, 40 the reaction will of course be carried out at a temperature above the melting point of the same. In any event, after the completion of the reaction the mixture is permitted to remain quiescent for a period, whereupon straitification ensues, 45 resulting in the formation of a lower aqueous layer containing the water soluble salt formed by the reaction, and simultaneously resulting in the formation of an upper hydrocarbon layer containing the copper soap dissolved therein. The 50 aqueous layer may be withdrawn and discarded, and the hydrocarbon layer, preferably after blowing or otherwise drying to free it from residual moisture, is ready for use as an impregnating medium. Material prepared in this way is homo- 55

- geneous, does not require centrifuging, and may easily be prepared with a copper content of at least 3%. The desirable features which have been specifically illustrated in application to the impregnation of paper, or to the manufacture of the hydrocarbon material containing the dissolved copper soap, are of course applicable generally to any application of the impregnating material to materials in the web.
- 10 The material is preferably applied to the web in fluid condition following the usual methods for impregnating with similar materials, such as paraffin and petrolatum. It is a further advantage of this process that it not only renders the material treated proof against fungi, but also makes it moisture proof.
- 15
- 10 The foregoing description is for purposes of illustration and not of limitation, and it is therefore my intention that the invention be limited only by the appended claims or their equivalents, 15 wherein I have endeavored to claim broadly all inherent novelty.

I claim:

1. A wrapping paper impregnated with petrolatum containing dissolved therein an oil soluble copper compound, and adapted to substantially permanently prevent the spreading of fungi from a point of fungus propagation, said paper being substantially permanently water-repellent and containing at least 1% of copper. 5
2. A wrapping paper impregnated with petrolatum containing dissolved therein copper oleate, 10 and copper resinate, and adapted to substantially permanently prevent the spreading of fungi from a point of fungus propagation, said paper being substantially permanently water-repellent, said copper oleate being present in the proportions of 15 from 25 to 75% of the total amount of copper oleate and copper resinate present, and the amount of hydrocarbon present ranging from one-third to three times the amount by weight of copper oleate and copper resinate. 20

LEO LIBERTHSON.